



US007582200B2

(12) **United States Patent**  
**Rosenbaum et al.**

(10) **Patent No.:** **US 7,582,200 B2**  
(45) **Date of Patent:** **Sep. 1, 2009**

(54) **HYDRAULIC SYSTEM AND A METHOD OF OPERATING A HYDRAULIC PUMP**

(75) Inventors: **John M. Rosenbaum**, Richmond, CA (US); **Susan M. Abernathy**, Hercules, CA (US); **Nancy J. Bertrand**, Lafayette, CA (US)

(73) Assignee: **Chevron U.S.A. Inc.**, San Ramon, CA (US)

(\*) Notice: Subject to any disclaimer, the term of this patent is extended or adjusted under 35 U.S.C. 154(b) by 0 days.

(21) Appl. No.: **12/165,180**

(22) Filed: **Jun. 30, 2008**

(65) **Prior Publication Data**

US 2008/0264053 A1 Oct. 30, 2008

**Related U.S. Application Data**

(63) Continuation-in-part of application No. 11/078,746, filed on Mar. 11, 2005, now Pat. No. 7,435,327.

(60) Provisional application No. 60/637,171, filed on Dec. 16, 2004.

(51) **Int. Cl.**

**C10G 71/00** (2006.01)

**C10M 175/00** (2006.01)

(52) **U.S. Cl.** ..... **208/18; 208/19; 208/180**

(58) **Field of Classification Search** ..... **208/180, 208/18, 19**  
See application file for complete search history.

(56) **References Cited**

U.S. PATENT DOCUMENTS

6,090,758 A 7/2000 Pillon et al.

6,103,099 A 8/2000 Wittenbrink et al.  
2008/0026968 A1 1/2008 Deckman et al.  
2008/0026969 A1 1/2008 Deckman et al.  
2008/0026970 A1 1/2008 Wright et al.  
2008/0026971 A1 1/2008 Deckman et al.

FOREIGN PATENT DOCUMENTS

WO WO00/14183 3/2000

OTHER PUBLICATIONS

Brendan Casey, "Moble Hydraulic Equipment: Increasing the Presure", Machinery Lubrication Magazine, Jan. 2008, 200801.

*Primary Examiner*—Walter D Griffin

*Assistant Examiner*—Frank C Campanell

(74) *Attorney, Agent, or Firm*—Susan M. Abernathy

(57) **ABSTRACT**

A method of operating a hydraulic pump, comprising:  
a. filling a hydraulic system oil reservoir with a hydraulic oil comprising:  
i. a lubricant base oil having defined properties; and  
ii. an antiwear hydraulic oil additive package; wherein the hydraulic oil has an air release at 50° C. less than 0.8 minutes; and  
b. operating the hydraulic pump without pump cavitation.

A hydraulic system, comprising a hydraulic system oil reservoir holding a hydraulic oil comprising:

- i. a lubricant base oil, optionally having defined properties; and
- ii. an antiwear hydraulic oil additive package; wherein the hydraulic oil has an air release at 50° C. less than 0.8 minutes.

In one embodiment the hydraulic oil additionally has low foam tendency and good demulsibility.

**20 Claims, No Drawings**

## 1

**HYDRAULIC SYSTEM AND A METHOD OF OPERATING A HYDRAULIC PUMP**

This application is a continuation-in-part, and it claims the benefit, of the co-pending prior nonprovisional application Ser. No. 11/078,746, filed Mar. 11, 2005; which is herein incorporated in its entirety. This application also claims the benefit of provisional Application No. 60/637,171, filed Dec. 16, 2004.

**FIELD OF THE INVENTION**

This invention is directed to a hydraulic system, and to a method of operating a hydraulic pump without pump cavitation.

**SUMMARY**

We provide a method of operating a hydraulic pump, comprising:

- a. filling a hydraulic system oil reservoir with a hydraulic oil comprising:
  - i. a lubricant base oil having:
    - 1) an average molecular weight greater than 475;
    - 2) a viscosity index greater than 140;
    - 3) a weight percent olefins less than 10; and
  - ii. an antiwear hydraulic oil additive package that is blended with the lubricant base oil; wherein the hydraulic oil has an air release at 50° C. by ASTM D 3427-03 of less than 0.8 minutes; and
- b. operating the hydraulic pump supplied with the hydraulic oil from the filled oil reservoir; wherein the hydraulic pump operates without pump cavitation.

We provide a hydraulic system, comprising a hydraulic system oil reservoir holding a hydraulic oil comprising:

- a. a lubricant base oil having:
  - i. an average molecular weight greater than 475;
  - ii. a viscosity index greater than 140;
  - iii. a weight percent olefins less than 10; and
- b. an antiwear hydraulic oil additive package that is blended with the lubricant base oil; wherein the hydraulic oil has an air release at 50° C. by ASTM D 3427-03 of less than 0.8 minutes.

We also provide a hydraulic system, comprising a hydraulic system oil reservoir holding a hydraulic oil comprising:

- a. a lubricant base oil, and
- b. an antiwear hydraulic oil additive package that is blended with the lubricant base oil; wherein the hydraulic oil has:
  - i. an air release at 50° C. by ASTM D 3427-03 of less than 0.8 minutes;
  - ii. a sequence II foam tendency by ASTM D 892-03 of less than 50 ml; and
  - iii. a number of minutes to 3 ml emulsion at 54° C. by ASTM D 1401-02 of less than 30.

**DETAILED DESCRIPTION**

Air release properties are generally associated with the base oil composition and kinematic viscosity. Air release properties are measured by ASTM D 3427-03. The air release test is done by saturating the fluid (normally at 50° C., but other temperatures such as 25° C. are also possible) with air bubbles and then measuring the time it takes for the fluid to return to an air content of 0.2%. Air release times are generally longer for Group I base oils than for Group III base oils.

## 2

Polyol ester, polyalphaolefin, and phosphate ester base oils typically have lower air release than conventional mineral oils. Typical air release specifications for hydraulic oils vary from 5 minutes maximum for ISO 32 oils, through 7 minutes maximum for ISO 46 oils, through 17 minutes maximum for ISO 150 oils. Air release values generally increase with viscosity of the base oil.

Good air release is a critical property for hydraulic oils. Agitation of hydraulic oil with air in equipment, such as bearings, couplings, gears, pumps, and oil return lines, may produce a dispersion of finely divided air bubbles in the oil. If the residence time in the hydraulic system reservoir is too short to allow the air bubbles to rise to the oil surface, a mixture of air and oil will circulate through the hydraulic system. This may result in an inability to maintain oil pressure, incomplete oil films in bearings and gears, and poor hydraulic system performance or failure. The inability to maintain oil pressure is especially pronounced with hydraulic systems having centrifugal pumps. Oil having poor air release can cause sponginess and lack of sensitivity of the control of turbine and hydraulic systems.

One of the most severe effects of a hydraulic oil having poor air release is pump cavitation. Cavitation of the hydraulic pump is evidenced primarily by increased pump noise and excessive pump vibration, and also by loss of high pressure in the hydraulic system or loss of speed in hydraulic system cylinders. When the hydraulic oil being pumped in a hydraulic system enters the pump inlet the pressure is significantly reduced. The greater the flow velocity through the pump the greater the pressure drop. If the pressure drop is high enough, and the hydraulic oil has poor air release, the air contained in the hydraulic oil is carried into the pump as small bubbles. As the hydraulic oil flow velocity decreases the fluid pressure increases, causing the air bubbles to suddenly collapse on the outer portions of the pump impeller. The formation of the air bubbles and their subsequent collapse is referred to as pump cavitation. The hydraulic pump may be seriously damaged by cavitation.

Air release is measured by ASTM D 3427-03. Compressed air is blown through the test oil, which has been heated to a temperature of 25 or 50° C. After the air flow is stopped, the time required for the air entrained in the oil to reduce in volume to 0.2% is recorded. The air release time is the number of minutes needed for air entrained in the oil to reduce in volume to 0.2% under the conditions of the test and at the specified temperature. Air release is mainly a function of the base stock, and oils need to be monitored for this. The air release of the hydraulic oil is very low, generally less than 0.8 minutes at 50° C., less than 0.5 minutes at 50° C., less than 0.3 minutes at 50° C., or less than 0.1 minutes at 50° C. Additionally, they can have an air release at 25° C. less than 10 minutes, less than 5 minutes, less than 2.5 minutes, less than 1 minutes, or less than 0.5 minutes.

Foam tendency and stability are measured by ASTM D 892-03. ASTM D 892-03 measures the foaming characteristics of a lubricating base oil at 24° C. and 93.5° C. It provides a means of empirically rating the foaming tendency and stability of the foam. The lubricating base oil, maintained at a temperature of 24° C., is blown with air at a constant rate for 5 minutes then allowed to settle for 10 minutes. The volume of foam, in ml, is measured at the end of both periods (sequence I). The foaming tendency is provided by the first measurement, the foam stability by the second measurement. The test is repeated using a new portion of the lubricating base oil at 93.5° C. (sequence II); however the settling time is reduced to one minute. For ASTM D 892-03 (sequence III) the same sample is used from sequence II, after the foam has

collapsed and cooled to 24° C. The lubricating base oil is blown with dry air for 5 minutes, and then settled for 10 minutes. The foam tendency and stability are again measured, and reported in ml. A good quality hydraulic oil will generally have less than 100 ml foam tendency for each of sequence I, II, and III; and zero ml foam stability for each of sequence I, II, III; the lower the foam tendency of a lubricating base oil or hydraulic oil the better. In one embodiment, the hydraulic oil has a much lower foaming tendency than typical hydraulic oils. In one embodiment the lubricant base oil has a sequence I foam tendency less than 50 ml; or a sequence II foam tendency less than 50 ml, or a sequence III foam tendency less than 30 ml. In another embodiment the lubricant base oil has a sequence III foam tendency less than 50 ml.

The antiwear additive may be an additive package provided by an additive company or formulated by a lubricant formulator. An example of an additive package is an AW hydraulic oil additive package, for example one that meets the Denison HF-0 standard. It may be an ashless, zinc-free, or a zinc-based AW hydraulic oil additive package. Some AW hydraulic oil additive packages designed to meet the Denison HF-0 standard will also meet the AFNOR wet filterability test. The Denison HF-0 standard concerns hydraulic oils for use in axial piston pumps and vane pumps in severe duty applications. The HF-0 standard specifies high thermal stability, good rust prevention, high hydrolytic stability, good oxidation stability, low foaming, excellent filterability with and without water, and satisfactory performance in proprietary Denison pump tests.

In addition the HF-0 standard specifies the hydraulic oil have a viscosity index greater than 90, and a minimum aniline point of 100° C. (212° F.). The requirements for the Denison HF-0 standard are summarized below.

| Denison HF-0 Standard            |                                     |                            |
|----------------------------------|-------------------------------------|----------------------------|
| Requirements                     | Method                              | HF-0                       |
| Viscosity Index                  | ASTM D 567                          | ≥90                        |
| Foam Test                        | ASTM D 892                          | None                       |
| Allowable foam after 10 minutes  |                                     |                            |
| Aniline Point, ° C.              |                                     | ≥100                       |
| Rust                             | ASTM D 665A<br>ASTM D 665B          | Pass<br>Pass               |
| Thermal Stability                | CINCINNATI                          |                            |
| Sludge, mg.                      | MILACRON Proc A.                    | ≤100                       |
| Copper Weight Loss, mg.          | (135° C., 168 hr)                   | ≤10                        |
| Copper rod rating                |                                     | Report                     |
| Hydrolytic Stability             | ASTM D 2619                         |                            |
| Copper Weight Loss, mg.          |                                     | ≤0.2                       |
| Water layer acidity, mg KOH/g    |                                     | ≤4.0                       |
| Filterability                    | Denison TP 02100                    |                            |
| Without water, seconds           |                                     | ≤600                       |
| With 2% water                    |                                     | ≤2 × time<br>without water |
| Oxidation (1000 hours)           | ASTM D 4310                         |                            |
| Acid Number, mg KOH/g            |                                     | ≤2.0                       |
| Total Sludge, mg                 |                                     | ≤200                       |
| Total metals in oil/water/sludge |                                     |                            |
| Copper, mg                       |                                     | ≤50                        |
| Iron, mg                         |                                     | ≤50                        |
| Denison Pump Tests               | DENISON Vane &<br>Axial Piston Pump | Satisfactory               |

Wet filterability may be measured by the Denison TP 02100 test method or the AFNOR NFE 48-691 standard. For example, only fluids passing AFNOR NFE 48-691 are specified for injection molding hydraulic oils. The latter test measures filtration in the presence of water for an aged oil, which more closely replicates actual operating conditions. The tests

measure the times taken to filter initial and subsequent volumes of oil, which are then used to calculate the Index of Filtration (IF). The closer the IF is to one, the lower the tendency to clog filters over time and therefore the more desirable the oil.

The number of minutes to 3 ml emulsion at 54° C. is a measure of the demulsibility of the hydraulic oil. Demulsibility is measured by ASTM D 1401-02. A 40-ml sample of oil and 40 ml of distilled water are put into a 100-ml graduate cylinder. The mixture is stirred for 5 minutes while maintained at a temperature of 130° F. The time required for separation of the emulsion into its oil and water components is recorded. If, at the end of 30 minutes, 3 or more milliliters of emulsion still remain, the test is discontinued and the milliliters of oil, water, and emulsion are reported. The 3 measurements are presented in that order and are separated by hyphens. Test time, in minutes, is shown in parenthesis. In one embodiment, the hydraulic oil has excellent demulsibility. That is, the number of minutes to 3 ml emulsion at 54° C. by 20 ASTM D 1401-02 can be less than 30 minutes, or less than 20 minutes.

Liquids that contain mixtures of different types of molecules result in the stabilization of thin layers of liquid at the air/liquid interface which slows the release of entrained air bubbles, thereby forming foam. Foaming will vary in different base oils but can be controlled by the addition of antifoam agents. Generally, the hydraulic oils will usually not require the addition of antifoam agents in addition to the hydraulic oil additive package. Most hydraulic oil additive packages 30 include antifoam agents. However, hydraulic oil blends of a higher viscosity or additionally comprising other base oils may exhibit foaming. Examples of antifoam agents are silicone oils, silicone polymers, mixtures of silicone fluid and silicone resin, silicone glycols, polyacrylates, polyacrylate esters, acrylic polymers, and fluorosilicones.

Antifoam agents work by destabilizing the liquid film that surrounds entrained air bubbles. To be effective they must spread effectively at the air/liquid interface. According to theory, the antifoam agent will spread if the value of the 40 spreading coefficient, S, is positive. S is defined by the following equation:  $S = p_1 - p_2 - p_{1,2}$ , wherein  $p_1$  is the surface tension of the foamy liquid,  $p_2$  is the surface tension of the antifoam agent, and  $p_{1,2}$  is the interfacial tension between them. Surface tension and interfacial tensions are measured 45 using a ring type tensiometer by ASTM D 1331-89, "Surface and Interfacial Tension of Solutions of Surface-Active Agents". As used herein,  $p_1$  is the surface of the hydraulic oil prior to the addition of antifoam agent.

In one embodiment, an antifoam agent is used when 50 blended into the hydraulic oil, exhibits a spreading coefficient of at least 2 mN/m at both 24° C. and 93.5° C. Various types of antifoam agents are taught, for example, in U.S. Pat. No. 6,090,758 and US20070112078. When used, the antifoam agents should not significantly increase the air release time of 55 the hydraulic oil. Another example of an antifoam agent is high molecular weight polydimethyl siloxane, a type of silicone antifoam agent. Another example of antifoam agent is an acrylate antifoam agent, which is less likely to adversely effect air release properties compared to lower molecular weight silicone antifoam agents.

In one embodiment, additives known for improving the air 60 release rate of lubricating compositions can be used in the hydraulic oil. These additives include vinyl aromatic-olefin block copolymer that forms a micelle-like structure when blended with the lubricant base oil. These copolymers are taught in U.S. Patent Publication US20080026969A1. Additives that improve air release also include alkyl salicylate

## 5

detergent, including ashless nitrogen-containing alkyl salicylate detergent. These detergents are taught in U.S. Patent Publication US20080026971A1.

In one embodiment, the hydraulic oil may include a thickener. Thickeners include both traditional thickeners and viscosity index (VI) improvers. Traditional thickeners include, for example, polyisobutylene (PIB) and high viscosity PAOs. Thickeners that are VI improvers include, for example, polymethacrylate, olefin co-polymer, styrene butadiene copolymers, styrene isoprene polymers, and SV Star polymers. The SV star polymers consist of a core (divinyl benzene) with arms of isoprene that radiate out from the core. When a thickener is blended into the hydraulic oil, the treat rate of the thickener and the lubricant base oil are chosen to achieve a favorable air release by using a relationship between the thickener, lubricant viscosity and viscosity of at least one lubricant base oil. The relationship may be represented by an algorithm. This relationship and algorithm are taught in U.S. Patent Publication US20080026970A1.

## Specific Analytical Test Methods:

## Wt % Olefins:

The wt % Olefins in the lubricant base oil is determined by proton-NMR by the following steps, A-D:

A. Prepare a solution of 5-10% of the test hydrocarbon in deuteriochloroform.

B. Acquire a normal proton spectrum of at least 12 ppm spectral width and accurately reference the chemical shift (ppm) axis. The instrument must have sufficient gain range to acquire a signal without overloading the receiver/ADC. When a 30 degree pulse is applied, the instrument must have a minimum signal digitization dynamic range of 65,000. In one embodiment, the dynamic range is 260,000 or more.

C. Measure the integral intensities between:

6.0-4.5 ppm (olefin)

2.2-1.9 ppm (allylic)

1.9-0.5 ppm (saturate)

D. Using the molecular weight of the test substance determined by ASTM D 2503, calculate:

1. The average molecular formula of the saturated hydrocarbons

2. The average molecular formula of the olefins

3. The total integral intensity (=sum of all integral intensities)

4. The integral intensity per sample hydrogen (=total integral/number of hydrogens in formula)

5. The number of olefin hydrogens (=Olefin integral/integral per hydrogen)

6. The number of double bonds (=Olefin hydrogen times hydrogens in olefin formula/2)

7. The wt % olefins by proton NMR=100 times the number of double bonds times the number of hydrogens in a typical olefin molecule divided by the number of hydrogens in a typical test substance molecule.

The wt % olefins by proton NMR calculation procedure, D, works best when the % olefins result is low, less than about 15 weight percent. The olefins must be "conventional" olefins; i.e. a distributed mixture of those olefin types having hydrogens attached to the double bond carbons such as: alpha, vinylidene, cis, trans, and trisubstituted. These olefin types will have a detectable allylic to olefin integral ratio between 1 and about 2.5. When this ratio exceeds about 3, it indicates a higher percentage of tri or tetra substituted olefins are present and that different assumptions must be made to calculate the number of double bonds in the sample.

## 6

## Aromatics Measurement by HPLC-UV:

The method used to measure low levels of molecules with at least one aromatic function in the lubricant base oil uses a Hewlett Packard 1050 Series Quaternary Gradient High Performance Liquid Chromatography (HPLC) system coupled with a HP 1050 Diode-Array UV-Vis detector interfaced to an HP Chem-station. Identification of the individual aromatic classes in the highly saturated lubricating base oils was made on the basis of their UV spectral pattern and their elution time.

- 10 The amino column used for this analysis differentiates aromatic molecules largely on the basis of their ring-number (or more correctly, double-bond number). Thus, the single ring aromatic containing molecules elute first, followed by the polycyclic aromatics in order of increasing double bond number per molecule. For aromatics with similar double bond character, those with only alkyl substitution on the ring elute sooner than those with naphthenic substitution.

Unequivocal identification of the various base oil aromatic hydrocarbons from their UV absorbance spectra was accom-

- 20 plished recognizing that their peak electronic transitions were all red-shifted relative to the pure model compound analogs to a degree dependent on the amount of alkyl and naphthenic substitution on the ring system. These bathochromic shifts are well known to be caused by alkyl-group delocalization of the  $\pi$ -electrons in the aromatic ring. Since few unsubstituted aromatic compounds boil in the lubricant range, some degree of red-shift was expected and observed for all of the principle aromatic groups identified.

Quantitation of the eluting aromatic compounds was made 30 by integrating chromatograms made from wavelengths optimized for each general class of compounds over the appropriate retention time window for that aromatic. Retention time window limits for each aromatic class were determined by manually evaluating the individual absorbance spectra of eluting compounds at different times and assigning them to the appropriate aromatic class based on their qualitative similarity to model compound absorption spectra. With few exceptions, only five classes of aromatic compounds were observed in highly saturated API Group II and III lubricant base oils.

## 40 HPLC-UV Calibration:

HPLC-UV is used for identifying these classes of aromatic compounds even at very low levels. Multi-ring aromatics typically absorb 10 to 200 times more strongly than single-ring aromatics. Alkyl-substitution also affected absorption by about 20%. Therefore, it is important to use HPLC to separate and identify the various species of aromatics and know how efficiently they absorb.

Five classes of aromatic compounds were identified. With 50 the exception of a small overlap between the most highly retained alkyl-1-ring aromatic naphthenes and the least highly retained alkyl naphthalenes, all of the aromatic compound classes were baseline resolved. Integration limits for the co-eluting 1-ring and 2-ring aromatics at 272 nm were 55 made by the perpendicular drop method. Wavelength dependent response factors for each general aromatic class were first determined by constructing Beer's Law plots from pure model compound mixtures based on the nearest spectral peak absorbances to the substituted aromatic analogs.

For example, alkyl-cyclohexylbenzene molecules in base oils exhibit a distinct peak absorbance at 272 nm that corresponds to the same (forbidden) transition that unsubstituted tetralin model compounds do at 268 nm. The concentration of alkyl-1-ring aromatic naphthenes in base oil samples was 60 calculated by assuming that its molar absorptivity response factor at 272 nm was approximately equal to tetralin's molar absorptivity at 268 nm, calculated from Beer's law plots.

Weight percent concentrations of aromatics were calculated by assuming that the average molecular weight for each aromatic class was approximately equal to the average molecular weight for the whole base oil sample.

This calibration method was further improved by isolating the 1-ring aromatics directly from the lubricant base oils via exhaustive HPLC chromatography. Calibrating directly with these aromatics eliminated the assumptions and uncertainties associated with the model compounds. As expected, the isolated aromatic sample had a lower response factor than the model compound because it was more highly substituted.

More specifically, to accurately calibrate the HPLC-UV method, the substituted benzene aromatics were separated from the bulk of the lubricant base oil using a Waters Semi-Preparative HPLC unit. 10 grams of sample was diluted 1:1 in n-hexane and injected onto an amino-bonded silica column, a 5 cm×22.4 mm ID guard, followed by two 25 cm×22.4 mm ID columns of 8-12 micron amino-bonded silica particles, manufactured by Rainin Instruments, Emeryville, Calif., with n-hexane as the mobile phase at a flow rate of 18 mls/min. Column eluent was fractionated based on the detector response from a dual wavelength UV detector set at 265 nm and 295 nm. Saturate fractions were collected until the 265 nm absorbance showed a change of 0.01 absorbance units, which signaled the onset of single ring aromatic elution. A single ring aromatic fraction was collected until the absorbance ratio between 265 nm and 295 nm decreased to 2.0, indicating the onset of two ring aromatic elution. Purification and separation of the single ring aromatic fraction was made by re-chromatographing the monoaromatic fraction away from the "tailing" saturates fraction which resulted from overloading the HPLC column.

This purified aromatic "standard" showed that alkyl substitution decreased the molar absorptivity response factor by about 20% relative to unsubstituted tetralin.

#### Confirmation of Aromatics by NMR:

The weight percent of all molecules with at least one aromatic function in the purified mono-aromatic standard was confirmed via long-duration carbon 13 NMR analysis. NMR was easier to calibrate than HPLC UV because it simply measured aromatic carbon so the response did not depend on the class of aromatics being analyzed. The NMR results were translated from % aromatic carbon to % aromatic molecules (to be consistent with HPLC-UV and D 2007) by knowing that 95-99% of the aromatics in highly saturated lubricant base oils were single-ring aromatics.

High power, long duration, and good baseline analysis were needed to accurately measure aromatics down to 0.2% aromatic molecules.

More specifically, to accurately measure low levels of all molecules with at least one aromatic function by NMR, the standard D 5292-99 method was modified to give a minimum carbon sensitivity of 500:1 (by ASTM standard practice E 386). A 15-hour duration run on a 400-500 MHz NMR with a 10-12 mm Nalorac probe was used. Acorn PC integration software was used to define the shape of the baseline and consistently integrate. The carrier frequency was changed once during the run to avoid artifacts from imaging the aliphatic peak into the aromatic region. By taking spectra on either side of the carrier spectra, the resolution was improved significantly.

#### Molecular Composition by FIMS:

The lubricant base oil was characterized by Field Ionization Mass Spectroscopy (FIMS) into alkanes and molecules with different numbers of unsaturations. The distribution of

the molecules in the oil fractions was determined by FIMS. The samples were introduced via solid probe, typically by placing a small amount (about 0.1 mg.) of the base oil to be tested in a glass capillary tube. The capillary tube was placed at the tip of a solids probe for a mass spectrometer, and the probe was heated from about 40 to 50° C. up to 500 or 600° C. at a rate between 50° C. and 100° C. per minute in a mass spectrometer operating at about 10<sup>-6</sup> torr. The mass spectrometer was scanned from m/z 40 to m/z 1000 at a rate of 5 seconds per decade.

The mass spectrometers used were a Micromass Time-of-Flight and a Micromass VG70VSE. Results from the two different instruments were assumed to be equivalent. Response factors for all compound types were assumed to be 1.0, such that weight percent was determined from area percent. The acquired mass spectra were summed to generate one "averaged" spectrum.

The lubricant base oil was characterized by FIMS into alkanes and molecules with different numbers of unsaturations. The molecules with different numbers of unsaturations may be comprised of cycloparaffins, olefins, and aromatics. If aromatics were present in significant amounts in the lubricant base oil they would be identified in the FIMS analysis as 4-unsaturations. When olefins were present in significant amounts in the lubricant base oil they would be identified in the FIMS analysis as 1-unsaturations. The total of the 1-unsaturations, 2-unsaturations, 3-unsaturations, 4-unsaturations, 5-unsaturations, and 6-unsaturations from the FIMS analysis, minus the wt % olefins by proton NMR, and minus the wt % aromatics by HPLC-UV is the total weight percent of molecules with cycloparaffinic functionality in the lubricant base oil. Note that if the aromatics content was not measured, it was assumed to be less than 0.1 wt % and not included in the calculation for total weight percent of molecules with cycloparaffinic functionality.

Molecules with cycloparaffinic functionality mean any molecule that is, or contains as one or more substituents, a monocyclic or a fused multicyclic saturated hydrocarbon group. The cycloparaffinic group may be optionally substituted with one or more substituents. Representative examples include, but are not limited to, cyclopropyl, cyclobutyl, cyclopentyl, cyclohexyl, cycloheptyl, cycloheptyl, decahydronaphthalene, octahydronaphthalene, (pentadecan-6-yl)cyclohexane, 3,7,10-tricyclohexylpentadecane, decahydro-1-(pentadecan-6-yl)naphthalene, and the like.

Molecules with monocycloparaffinic functionality mean any molecule that is a monocyclic saturated hydrocarbon group of three to seven ring carbons or any molecule that is substituted with a single monocyclic saturated hydrocarbon group of three to seven ring carbons. The cycloparaffinic group may be optionally substituted with one or more substituents. Representative examples include, but are not limited to, cyclopropyl, cyclobutyl, cyclopentyl, cyclohexyl, cycloheptyl, (pentadecan-6-yl)cyclohexane, and the like.

Molecules with multicycloparaffinic functionality mean any molecule that is a fused multicyclic saturated hydrocarbon ring group of two or more fused rings, any molecule that is substituted with one or more fused multicyclic saturated hydrocarbon ring groups of two or more fused rings, or any molecule that is substituted with more than one monocyclic saturated hydrocarbon group of three to seven ring carbons. The fused multicyclic saturated hydrocarbon ring group in one embodiment is of two fused rings. The cycloparaffinic group may be optionally substituted with one or more substituents. Representative examples include, but are not limited to, cyclohexyl, cycloheptyl, cyclooctyl, cyclohexyl, cycloheptyl, cyclooctyl, (pentadecan-6-yl)cyclohexane, and the like.

ited to, decahydronaphthalene, octahydronaphthalene, 3,7,10-tricyclohexylpentadecane, decahydro-1-(pentadecan-6-yl) naphthalene, and the like.

Alkyl Branches per 100 Carbons:

The branching properties of the lubricant base oil was determined by analyzing a sample of oil using carbon-13 NMR according to the following seven-step process. References cited in the description of the process provide details of the process steps. Steps 1 and 2 are performed only on the initial materials from a new process.

- 1) Identify the CH branch centers and the  $\text{CH}_3$  branch termination points using the DEPT Pulse sequence (Doddrell, D. T.; D. T. Pegg; M. R. Bendall, *Journal of Magnetic Resonance* 1982, 48, 323ff.).
- 2) Verify the absence of carbons initiating multiple branches (quaternary carbons) using the APT pulse sequence (Patt, S. L.; J. N. Shoolery, *Journal of Magnetic Resonance* 1982, 46, 535ff.).
- 3) Assign the various branch carbon resonances to specific branch positions and lengths using tabulated and calculated values (Lindeman, L. P., *Journal of Qualitative Analytical Chemistry* 43, 1971 1245ff; Netzel, D. A., et. al., *Fuel*, 60, 1981, 307ff).

EXAMPLES

| Branch           | NMR Chemical Shift (ppm) |
|------------------|--------------------------|
| 2-methyl         | 22.5                     |
| 3-methyl         | 19.1 or 11.4             |
| 4-methyl         | 14.0                     |
| 4+methyl         | 19.6                     |
| Internal ethyl   | 10.8                     |
| Propyl           | 14.4                     |
| Adjacent methyls | 16.7                     |

- 4) Quantify the relative frequency of branch occurrence at different carbon positions by comparing the integrated intensity of its terminal methyl carbon to the intensity of a single carbon (=total integral/number of carbons per molecule in the mixture). For the unique case of the 2 methyl branch, where both the terminal and the branch methyl occur at the same resonance position, the intensity was divided by two before doing the frequency of branch occurrence calculation. If the 4-methyl branch fraction is calculated and tabulated, its contribution to the 4-methyls must be subtracted to avoid double counting.
- 5) Calculate the average carbon number. The average carbon number may be determined with sufficient accuracy for lubricant materials by dividing the molecular weight of the sample by 14 (the formula weight of  $\text{CH}_2$ ).
- 6) The number of branches per molecule is the sum of the branches found in step 4.
- 7) The number of alkyl branches per 100 carbon atoms is calculated from the number of branches per molecule (step 6) times 100 divided by the average carbon number.

Branching measurements can be performed using any Fourier Transform NMR spectrometer. In one embodiment, the measurements are performed using a spectrometer having a magnet of 7.0 T or greater. In all cases, after verification by Mass Spectrometry, UV or an NMR survey that aromatic carbons were absent, the spectral width was limited to the saturated carbon region, about 0-80 ppm vs. TMS (tetramethylsilane). Solutions of 15-25 percent by weight in chloroform-d1 were excited by 45 degrees pulses followed by a 0.8

sec acquisition time. In order to minimize non-uniform intensity data, the proton decoupler was gated off during a 10 sec delay prior to the excitation pulse and on during acquisition. Total experiment times ranged from 11-80 minutes. The 5 DEPT and APT sequences were carried out according to literature descriptions with minor deviations described in the Varian or Bruker operating manuals.

DEPT is Distortionless Enhancement by Polarization Transfer. DEPT does not show quaternaries. The DEPT 45 10 sequence gives a signal for all carbons bonded to protons. DEPT 90 shows CH carbons only. DEPT 135 shows CH and  $\text{CH}_3$  up and  $\text{CH}_2$  180 degrees out of phase (down). APT is Attached Proton Test. It allows all carbons to be seen, but if CH and  $\text{CH}_3$  are up, then quaternaries and  $\text{CH}_2$  are down. The 15 sequences are useful in that every branch methyl should have a corresponding CH. And the methyls are clearly identified by chemical shift and phase. Both are described in the references cited. The branching properties of each sample were determined by C-13 NMR using the assumption in the calculations 20 that the entire sample was isoparaffinic. Corrections were not made for n-paraffins or cycloparaffins, which may have been present in the oil samples in varying amounts. The cycloparaffins content was measured using FIMS.

Boiling Range Distribution:

25 Lubricant base oils made by hydroisomerization dewaxing a waxy feed may comprise a mixture of varying molecular weights having a wide boiling range. This disclosure will refer to the 10 percent point and the 90 percent point of the respective boiling ranges. The 10 percent point refers to that 30 temperature at which 10 weight percent of the hydrocarbons present within that cut will vaporize at atmospheric pressure. Similarly, the 90 percent point refers to the temperature at which 90 weight percent of the hydrocarbons present will 35 vaporize at atmospheric pressure. In this disclosure when referring to boiling range distribution, the boiling range between the 10 percent and 90 percent boiling points is what is being referred to. For samples having a boiling range above 40 1000° F., the boiling range distributions in this disclosure were measured using the standard analytical method ASTM D 6352 or its equivalent. For samples having a boiling range below 1000° F., the boiling range distributions in this disclosure were measured using the standard analytical method ASTM D 2887 or its equivalent.

45 Process to Make the Lubricant Base Oil:

In one embodiment the feeds used to prepare the lubricant base oil are waxy feeds containing greater than 75 weight 50 percent normal paraffins, such as at least 85 weight percent normal paraffins, or at least 90 weight percent normal paraffins. The waxy feed may be a conventional petroleum derived feed, such as, for example, slack wax, or it may be derived 55 from a synthetic feed, such as, for example, a feed prepared from a Fischer-Tropsch synthesis. A major portion of the feed should boil above 650° F. In one embodiment, at least 80 weight percent (or at least 90 weight percent) of the feed will 60 boil above 650° F. In one embodiment, the highly paraffinic feeds used to prepare the lubricant base oil have an initial pour point above 0° C., or above 10° C.

Slack wax can be obtained from conventional petroleum 60 derived feedstocks by either hydrocracking or by solvent refining of the lube oil fraction. Typically, slack wax is recovered from solvent dewaxing feedstocks prepared by one of these processes. Hydrocracking is usually preferred because hydrocracking will also reduce the nitrogen content to a low 65 value. With slack wax derived from solvent refined oils, deoiling may be used to reduce the nitrogen content. Hydrotreating of the slack wax can be used to lower the nitrogen and sulfur

content. Slack waxes posses a very high viscosity index, normally in the range of from about 140 to 200, depending on the oil content and the starting material from which the slack wax was prepared. Therefore, slack waxes are suitable for the preparation of lubricant base oils having a very high viscosity index.

In one embodiment, the waxy feed has less than 25 ppm total combined nitrogen and sulfur. Nitrogen is measured by melting the waxy feed prior to oxidative combustion and chemiluminescence detection by ASTM D 4629-96. The test method is further described in U.S. Pat. No. 6,503,956, incorporated herein. Sulfur is measured by melting the waxy feed prior to ultraviolet fluorescence by ASTM D 5453-00. The test method is further described in U.S. Pat. No. 6,503,956, incorporated herein.

Waxy feeds are expected to be plentiful and relatively cost competitive in the near future as large-scale Fischer-Tropsch synthesis processes come into production. Syncrude prepared from the Fischer-Tropsch process comprises a mixture of various solid, liquid, and gaseous hydrocarbons. Those Fischer-Tropsch products which boil within the range of lubricant base oil contain a high proportion of wax which makes them ideal candidates for processing into lubricant base oil. Accordingly, Fischer-Tropsch wax represents an excellent feed for preparing high quality lubricant base oils. Fischer-Tropsch wax is normally solid at room temperature and, consequently, displays poor low temperature properties, such as pour point and cloud point. However, following hydroisomerization of the wax, Fischer-Tropsch derived lubricant base oils having excellent low temperature properties may be prepared. A general description of the hydroisomerization dewaxing process may be found in U.S. Pat. Nos. 5,135,638, 5,282,958, and 7,282,134, incorporated herein.

The hydroisomerization is achieved by contacting the waxy feed with a hydroisomerization catalyst in an isomerization zone under hydroisomerizing conditions. In one embodiment the hydroisomerization catalyst comprises a shape selective intermediate pore size molecular sieve, a noble metal hydrogenation component, and a refractory oxide support. In one embodiment, the shape selective intermediate pore size molecular sieve is selected from the group consisting of SAPO-11, SAPO-31, SAPO-41, SM-3, ZSM-22, ZSM-23, ZSM-35, ZSM-48, ZSM-57, SSZ-32, offretite, ferrierite, and combinations thereof. SAPO-11, SM-3, SSZ-32, ZSM-23, and combinations thereof are more preferred. In one embodiment, the noble metal hydrogenation component is platinum, palladium, or combinations thereof.

In one embodiment, the hydroisomerizing conditions depend on the waxy feed used, the hydroisomerization catalyst used, whether or not the catalyst is sulfided, the desired yield, and the desired properties of the lubricant base oil. Some hydroisomerization conditions that may be useful include temperatures of 260° C. to about 413° C. (500 to about 775° F.), a total pressure of 15 to 3000 psig, and a hydrogen to feed ratio from about 0.5 to 30 MSCF/bbl, or from about 1 to about 10 MSCF/bbl.

In one embodiment, the hydroisomerization conditions are tailored to produce one or more fractions having greater than 5 weight percent molecules with monocycloparaffinic functionality, such as having greater than 10 weight percent molecules with monocycloparaffinic functionality. In one embodiment the fractions will have a viscosity index greater than 140 and a pour point less than zero degrees C. In another embodiment, the pour point will be less than -10° C.

Optionally, the lubricant base oil produced by hydroisomerization dewaxing may be hydrofinished. The hydrofinishing may occur in one or more steps, either before or after

fractionating of the lubricant base oil into one or more fractions. The hydrofinishing is intended to improve the oxidation stability, UV stability, and appearance of the product by removing aromatics, olefins, color bodies, and solvents. A general description of hydrofinishing may be found in U.S. Pat. Nos. 3,852,207 and 4,673,487, incorporated herein. In one embodiment, the hydrofinishing step may be used to reduce the weight percent olefins in the lubricant base oil to less than 10, less than 5, less than 1, or less than 0.5. The hydrofinishing step may also be used to reduce the weight percent aromatics to less than 0.3, less than 0.06, less than 0.02, or less than 0.01.

In one embodiment, the hydroisomerizing and hydrofinishing conditions are tailored to produce one or more selected fractions of lubricant base oil having less than 0.06 weight percent aromatics, less than 5 weight percent olefins, and greater than 5 weight percent molecules with cycloparaffinic functionality.

In one embodiment, the lubricant base oil has an average molecular weight greater than 475, such as in a range between about 500 and about 900. Molecular weight is measured by ASTM D 2503, but other methods giving comparable results (such as ASTM D 2502) may also be used. In one embodiment, the lubricant base oil has a very high viscosity index, such as greater than 140, or greater than an amount calculated by the equation: Viscosity Index=28xLn (Kinematic Viscosity at 100° C., in cSt)+95; wherein Ln refers to the natural logarithm to the base 'e'. Viscosity index is determined by ASTM D 2270-93 (1998).

In one embodiment, the lubricant base oil has measurable quantities of unsaturated molecules measured by FIMS. For example, it may have greater than 5 weight percent (or greater than 10 weight percent) molecules with monocycloparaffinic functionality. In another embodiment, the lubricant base oil can have a ratio of weight percent molecules with monocycloparaffin functionality to weight percent molecules with multicycloparaffinic functionality greater than 6, such as greater than 15, or greater than 40. The presence of predominantly molecules with monocycloparaffinic functionality in the lubricant base oil fractions provides excellent oxidation stability as well as desired additive solubility and elastomer compatibility.

In one embodiment, the lubricant base oil has a weight percent olefins less than 10, less than 5, less than 1, or less than 0.5. In another embodiment the lubricant base oil has a weight percent aromatics less than 0.3, less than 0.06, or less than 0.02.

In one embodiment the lubricant base oil has low levels of alkyl branches per 100 carbons, such as less than 8 or less than 7 alkyl branches per 100 carbons. The alkyl branches may be predominantly methyl branches ( $-\text{CH}_3$ ). In addition, the alkyl branches may be positioned over various branch carbon resonances by carbon-13 NMR. Low levels of predominantly methyl branches impart high viscosity index and good biodegradability to the lubricating base oil, and the hydraulic oil made from it.

In one embodiment, the lubricant base oil will have T90-T10 boiling point distribution less than 180° F., such as between 50° F. and less than 180° F., or between 90 and less than 150° F.

In one embodiment, the Oxidator BN of the lubricant base oil will be greater than 25 hours, such as greater than 35 hours, or greater than 40 hours. Oxidator BN is a convenient way to measure the oxidation stability of lubricating base oils. The Oxidator BN test is described by Stangeland et al. in U.S. Pat. No. 3,852,207. The Oxidator BN test measures the resistance to oxidation by means of a Dornte-type oxygen absorption

apparatus. See R. W. Dornte "Oxidation of White Oils," Industrial and Engineering Chemistry, Vol. 28, page 26, 1936. Normally, the conditions are one atmosphere of pure oxygen at 340° F. The results are reported in hours to absorb 1000 ml of O<sub>2</sub> by 100 g. of oil. In the Oxidator BN test, 0.8 ml of catalyst is used per 100 grams of oil and an additive package is included in the oil. The catalyst is a mixture of soluble metal naphthenates in kerosene. The mixture of soluble metal naphthenates simulates the average metal analysis of used crankcase oil. The level of metals in the catalyst is as follows: Copper=6,927 ppm; Iron=4,083 ppm; Lead=80,208 ppm; Manganese=350 ppm; Tin=3565 ppm. The additive package is 80 millimoles of zinc bispolypolypropylenephenyldithio-phosphate per 100 grams of oil, or approximately 1.1 grams of OLOA 260. The Oxidator BN test measures the response of a lubricating base oil in a simulated application. High values, or long times to absorb one liter of oxygen, indicate good oxidation stability. Traditionally it is considered that the Oxidator BN should be above 7 hours.

OLOA is an acronym for Oronite Lubricating Oil Additive®, which is a registered trademark of Chevron Oronite.

#### Hydraulic Pump Operation:

Hydraulic oil reservoirs must be filled to a sufficient volume to provide adequate lubrication, sufficient pressure head, and good coverage of pump suction inlets. Most hydraulic oil systems are marked with minimum fill lines. In general, the oil reservoir should be filled with hydraulic oil to the level indicated by the system operation manual, to a marked fill line, or to a minimum level (for example, about 3 inches) above the top of the highest pump suction inlet when all hydraulic system cylinders are fully extended.

Hydraulic oil reservoirs are sized and designed such that there is adequate residence time for the hydraulic fluid to release air and bubbles. When a hydraulic oil has improved air release, less tendency to form foam and very low foam stability, the hydraulic system may be designed with smaller oil reservoirs or less oil residence time. It may not be as critical that the oil reservoir be filled to the level indicated by the system operation manual.

Even with a small oil reservoir or shorter oil residence time the hydraulic pump may be operated without cavitation when the hydraulic oil has excellent air release and foaming properties. This can be very useful where space is limited. Examples of where space could be limited are in aircraft, elevator, mobile equipment, or other hydraulic systems where space and weight are significant considerations.

Some hydraulic system designs include dynamic flow channels on the hydraulic oil's return path that allow for a smaller oil reservoir.

Examples of mobile equipment having hydraulic systems are marine equipment, forest machinery, mining machinery, agricultural machinery, construction machinery, earth moving machinery, fitness equipment, lawn and garden equipment, loading machinery, custom cars, and demolition machinery. Marine equipment is used by a wide variety of industries, such as offshore oil & gas, and national defense. Marine equipment is used for a number of activities, including for example: oceanographic research, seismic applications, shipping and transport, fisheries, and recreation. Examples of hydraulic systems on marine equipment are: cranes, bow & stern thrusters, winches, capstans, pressure switches, heat exchangers, wheel drives, guages, motors, accumulators, brakes, cylinders, jacks, presses, pullers, nail guns, filters, gear boxes, power units, power steering systems, and scales.

Hydraulics are used in forest machinery for loading and controlling timber, for example. Hydraulics are used in mining machinery for drilling, crushing, hammering, packing, loading, etc. Hydraulics are used in a wide variety of agricultural machinery, including hay beds, chippers, combines, pickers, harvesters, pruners, balers, packers, planters, sprayers, sweepers, coil packers, dryers, weighing scales, and livestock feeders. Hydraulics are used in construction machinery such as jacks, heavy-duty metal cutting shears, grapples, concrete breakers, spike drivers, and rail saws. Hydraulics are used in earth moving machinery such as earthmovers, scrapers, excavators, shovels, and loaders. Examples of loading machinery are trucks with shovels or buckets, pallet lifters, cranes, hoists, etc. Examples of demolition machinery are scrap cutters, crushers, packers, heavy-duty metal shears, lifts, and loaders.

Hydraulic pumps may be operated at higher pump speeds when they are operated with a hydraulic oil having improved air release and foaming tendency. The flow rate or capacity of a hydraulic pump is directly proportional to the pump speed; the discharge head is directly proportional to the square of the pump speed; and the power required by the pump motor is directly proportional to the cube of the pump speed. In a hydraulic system, the power available to do work is a product of the hydraulic oil flow rate (proportional to pump speed) and the hydraulic system pressure.

In one embodiment, the hydraulic oil is factory-filled into the hydraulic system. This can provide ease of use to the end-user. In some embodiments the hydraulic oil has an extended life and does not need to be changed out during the operating life of the equipment.

In one embodiment the hydraulic system is designed to produce very high power. This is achieved by increasing the hydraulic pump flow, increasing the average operating pressure, or a combination of both. The average operating pressure can vary between about 150 bar to about 500 bar, about 300 bar to about 500 bar, or about 400 bar to about 475 bar.

The invention will be further explained by the following illustrative examples that are intended to be non-limiting.

#### EXAMPLES

##### Example 1

45 A sample of hydrotreated Fischer-Tropsch wax made using a Fe-based Fischer-Tropsch catalyst was analyzed and found to have the properties as shown in Table I.

TABLE I

##### Fischer-Tropsch Wax

| Fischer-Tropsch Catalyst           | Fe-Based |
|------------------------------------|----------|
| Sulfur, ppm                        | <2       |
| Nitrogen, ppm                      | <8       |
| Oxygen by Neutron Activation, Wt % | 0.15     |
| Oil Content, D 721, Wt %           | <1       |
| GC N-Paraffin Analysis             |          |
| Total Normal Paraffin, Wt %        | 92.15    |
| Average Carbon Number              | 41.6     |
| Average Molecular Weight           | 585.4    |
| D 6352 SIMDIST TBP (WT %), °F.     |          |
| T0.5                               | 784      |
| T5                                 | 853      |
| T10                                | 875      |
| T20                                | 914      |
| T30                                | 941      |

TABLE I-continued

| Fischer-Tropsch Wax      |          |
|--------------------------|----------|
| Fischer-Tropsch Catalyst | Fe-Based |
| T40                      | 968      |
| T50                      | 995      |
| T60                      | 1013     |
| T70                      | 1031     |
| T80                      | 1051     |
| T90                      | 1081     |
| T95                      | 1107     |
| T99.5                    | 1133     |
| T90 – T10, °C.           | 114.5    |
| Wt % C30+                | 96.9     |
| Wt % C60+                | 0.55     |
| C60+/C30+                | 0.01     |

The Fischer-Tropsch wax was hydroisomerized over a Pt/SAPO-11 catalyst with an alumina binder. Operating conditions included temperatures between 652° F. and 695° F. (315° C. and 399° C.), LHSV of 0.6 to 1.0 hr<sup>-1</sup>, reactor pressure of 1000 psig, and once-through hydrogen rates of between 6 and 7 MSCF/bbl. The reactor effluent passed directly to a second reactor containing a Pt/Pd on silica-alumina hydrofinishing catalyst also operated at 1000 psig. Conditions in the second reactor included a temperature of 450° F. (232° C.) and an LHSV of 1.0 hr<sup>-1</sup>.

The products boiling above 650° F. were fractionated by vacuum distillation to produce distillate fractions of different viscosity grades. Three Fischer-Tropsch derived lubricant base oils were obtained. Two were distillate side-cut fractions (FT-4.5 and FT-6.3) and one was a distillate bottoms fraction (FTB-9.8). FTB-9.8 was an example of the lubricant base oils that are useful in this invention. The FIMS analyses were conducted on a Micromass VG70VSE mass spectrometer. The probe in the spectrophotometer was heated from about 40 to 500° C. at a rate of 50° C. per minute. Test data on the three Fischer-Tropsch derived lubricant base oils are shown in Table II, below.

TABLE II

| Fischer-Tropsch Derived Lubricant Base Oils   |        |        |         |
|-----------------------------------------------|--------|--------|---------|
| Properties                                    | FT-4.5 | FT-6.3 | FTB-9.8 |
| Viscosity at 100° C., cSt                     | 4,524  | 6,295  | 9,83    |
| Viscosity Index                               | 149    | 154    | 163     |
| Average Molecular Weight, ASTM D2503 or D2502 | 420    | 470    | 538     |
| Wt % Aromatics                                | 0.0109 | 0.0141 | 0.0162  |
| Wt % Olefins by Proton NMR                    | 1.1    | 0.40   | 0.0     |
| Formula Olefin H                              | 59.7   | 66.9   | 86.6    |
| Saturate H                                    | 61.7   | 68.9   | 88.6    |
| Total Integral div/H                          | 3058   | 8026   | —       |
| Olefin integral                               | 49.55  | 116.56 | 0.054   |
| Olefin H                                      | 1.14   | 1.0    | —       |
| Sample olefin H                               | 0.023  | 0.009  | 0.0     |
| Aniline Point, °F.                            | 253.2  | 263.0  | 278.6   |
| NMR - Alkyl branches per 100 carbons          | 7.48   | 7.21   | 6.63    |

TABLE II-continued

| Fischer-Tropsch Derived Lubricant Base Oils |        |        |         |       |
|---------------------------------------------|--------|--------|---------|-------|
| Properties                                  | FT-4.5 | FT-6.3 | FTB-9.8 |       |
| FIMS, Wt % of Molecules                     |        |        |         |       |
| Alkanes                                     | 89.4   | 76.0   | 81.3    |       |
| 1-Unsaturations                             | 10.4   | 22.1   | 16.4    |       |
| 2-6-Unsaturations                           | 0.2    | 1.9    | 2.3     |       |
| Total                                       | 100.0  | 100.0  | 100.0   |       |
| Total Wt % of Molecules                     | 9.49   | 23.59  | 18.68   |       |
| Having Cycloparaffinic Functionality        |        |        |         |       |
| Ratio of Molecules with                     | 48.9   | 11.5   | 7.2     |       |
| Monocycloparaffinic Functionality to        |        |        |         |       |
| Molecules with Multicycloparaffinic         |        |        |         |       |
| Functionality                               |        |        |         |       |
| SIMDIS (Wt %), °F.                          |        |        |         |       |
| 5                                           | 5      | 716    | 827     | 911   |
| 10                                          | 10     | 732    | 841     | 921   |
| 20                                          | 20     | 763    | 863     | 936   |
| 30                                          | 30     | 792    | 881     | 948   |
| 50                                          | 50     | 843    | 912     | 971   |
| 70                                          | 70     | 883    | 943     | 999   |
| 90                                          | 90     | 917    | 982     | 1050  |
| 95                                          | 95     | 929    | 996     | 1074  |
| Boiling Range Distribution                  |        | 185    | 87      | 129   |
| T90 – T10                                   |        |        |         |       |
| Oxidator BN, hours                          |        | 34.92  | 29.62   | 35.12 |

## Example 2

The Fischer-Tropsch derived lubricant base oils prepared above (FT-4.5, FT-6.3, and FTB-9.8) were blended with either a zinc antiwear hydraulic oil additive package designed to meet Denison HF-0 and AFNOR NFE 48-691 wet filterability standards or an ashless antiwear hydraulic oil additive package designed to meet Denison HF-0. A comparison blend with polyalphaolefin base oil and the zinc antiwear hydraulic oil additive package designed to meet HF-0 and AFNOR NFE 48-691 wet filterability standards was also prepared. All of these blends were ISO 32 grade. The compositions of the hydraulic oils are shown below in Table III.

TABLE III

| Composition of Hydraulic Oils from Fe-Based Fischer-Tropsch Wax |       |       |                   |                   |
|-----------------------------------------------------------------|-------|-------|-------------------|-------------------|
| Component                                                       | Oil 1 | Oil 2 | Comparative Oil 3 | Comparative Oil 4 |
| FTB-9.8                                                         | 99.15 | 98.75 | 0                 |                   |
| FT-4.5                                                          |       |       | 49.575            |                   |
| FT-6.3                                                          |       |       | 49.575            |                   |
| Polyalphaolefin Base Oil                                        |       |       | 0                 | 99.15             |
| Zinc Antiwear HF-0 Additive Package                             | 0.85  | 0     | 0.85              | 0.85              |
| Ashless Antiwear HF-0 Additive Package                          | 0     | 1.25  | 0                 | 0                 |

Oils 1 and 2 both comprise: 1) a lubricant base oil (FT-9.8) having: an average molecular weight greater than 475, a VI greater than 140, a weight percent olefins less than 10; and 2) an antiwear hydraulic oil additive package. The lubricant base oil used in Oils 1 and 2 had a level of less than about 8 alkyl branches per 100 carbons, which would give these hydraulic oils improved biodegradability.

The hydraulic oils were tested in a number of tests related to hydraulic oil performance. Storage stability tests were used to observe the additive solvencies over a 4 week period. The

storage conditions were room temperature (approximately 25° C.), 65° C., 0° C., or -18° C. The additive solvency observations were made at both the test temperatures, and (after warming, when required) at room temperature. The results of these tests are summarized in Table IV.

TABLE IV

| Properties                   | ISO 32 Hydraulic Oils |            |                   |                   |
|------------------------------|-----------------------|------------|-------------------|-------------------|
|                              | Oil 1                 | Oil 2      | Comparative Oil 3 | Comparative Oil 4 |
| <u>Air Release (D 3427)</u>  |                       |            |                   |                   |
| 50° C.                       | <0.1                  | Not tested | 1.3               | 1.0               |
| 25° C.                       | 2.4                   | Not tested | Not tested        | Not tested        |
| Demulsibility (D 1401)       | 39-40-1               | Not tested | 7-36-37           | 40-40-0           |
| Oil-Water-Emulsion (minutes) | (15)                  | tested     | (30)              | (10)              |
| Foam (D 892)                 |                       |            |                   |                   |
| Seq I                        | 10-0                  | Not tested | 110-0             | 20-0              |
| Seq II                       | 0-0                   | 20-0       | 20-0              |                   |
| Seq III                      | 10-0                  | 90-0       | 20-0              |                   |
| <u>Storage Stability</u>     |                       |            |                   |                   |
| RT @ 4 Wks                   | C                     | C          | C                 | C                 |
| 65° C. @ 4 Wks               | C                     | C          | C                 | C                 |
| 0° C. at RT @ 4 Wks          | C                     | C          | Sep.              | C                 |
| -18° C. at RT @ 4 Wks        | C                     | C          | C                 | C + T             |
| Storage Stability Codes      | C = clear             | C = clear  | Sep. = separated  | T = trace of haze |

The air release properties of Oil 1 were better than for Comparative Oil 3; which also comprised Fischer-Tropsch derived lubricant base oils. Neither of the base oils used in Comparative Oil 3 had an average molecular weight greater than 475. The air release properties of Oil 1 were also better than a high performance hydraulic oil made with polyalphaolefin base oil (Oil 4). The excellent additive solubility of Oils 1 and 2 is attributed to the cycloparaffin composition of the lubricant base oil used in these blends (FT-9.8). The FT-9.8 has greater than 5 weight percent molecules with cycloparaffinic functionality and the ratio of molecules with monocycloparaffinic functionality to molecules with multicycloparaffinic functionality is greater than 6. The hydraulic oils having the Fischer-Tropsch derived lubricant base oil with the highest molecular weight and highest aniline point showed the best air release, additive solubility, and foaming tendencies. Typically, better air release is expected with lower viscosity (thus lower molecular weight) base oil, and typically better additive solubility is expected with base oils having lower aniline points.

### Example 3

A wax sample composed of several different batches of hydrotreated Fischer-Tropsch wax, all made using a Co-based Fischer-Tropsch catalyst was prepared. The different batches of wax composing the wax sample were analyzed and all found to have the properties as shown in Table V.

TABLE V

| Fischer-Tropsch Wax      |          |
|--------------------------|----------|
| Fischer-Tropsch Catalyst | Co-Based |
| Sulfur, ppm              | <10      |
| Nitrogen, ppm            | <10      |

TABLE V-continued

| Fischer-Tropsch Wax             |           |
|---------------------------------|-----------|
| Fischer-Tropsch Catalyst        | Co-Based  |
| Oxygen, wt %                    | <0.50     |
| Wt % N-Paraffins by GC          | >85       |
| D 6352 SIMDIST TBP (Wt %), ° F. |           |
| 10 T10                          | 550-700   |
| 10 T90                          | 1000-1080 |
| T90 - T10, ° C.                 | >154      |

The Co-based Fischer-Tropsch wax was hydroisomerized over a Pt/SAPO-11 catalyst with an alumina binder. Operating conditions included temperatures between 635° F. and 675° F. (335° C. and 358° C.), LHSV of 1.0 hr<sup>-1</sup>, reactor pressure of about 500 psig, and once-through hydrogen rates of between 5 and 6 MSCF/bbl. The reactor effluent passed directly to a second reactor containing a Pd on silica-alumina hydrofinishing catalyst also operated at 500 psig. Conditions in the second reactor included a temperature of about 350° F. (177° C.) and an LHSV of 2.0 hr<sup>-1</sup>.

The products boiling above 650° F. were fractionated by vacuum distillation to produce two distillate fractions of different viscosity grades. They were both distillate side-cut fractions (FT-6.4 and FT-9.7). The FIMS analysis was conducted on a Micromass Time-of-Flight spectrophotometer. The emitter on the Micromass Time-of-Flight was a Carbotec 5 um emitter designed for FI operation. A constant flow of pentafluorochlorobenzene, used as lock mass, was delivered into the mass spectrometer via a thin capillary tube. The probe was heated from about 50° C. up to 600° C. at a rate of 100° C. per minute. Test data on the two Fischer-Tropsch derived lubricant base oils are shown in Table VI, below.

TABLE VI

| Fischer-Tropsch Derived Lubricant Base Oils                                                                    |        |            |
|----------------------------------------------------------------------------------------------------------------|--------|------------|
| Properties                                                                                                     | FT-6.4 | FT-9.7     |
| Viscosity at 100° C., cSt                                                                                      | 6.362  | 9.716      |
| Viscosity Index                                                                                                | 153    | 161        |
| Average Molecular Weight                                                                                       | 518    | 582        |
| Wt % Aromatics                                                                                                 | 0.059  | Not tested |
| Wt % Olefins                                                                                                   | 3.5    | 12.9       |
| Aniline Point, ° F.                                                                                            | 263    | Not tested |
| NMR - Alkyl branches per 100 carbons                                                                           | 10.13  | 7.56       |
| FIMS, Wt % of Molecules                                                                                        |        |            |
| Alkanes                                                                                                        | 68.1   | 60.9       |
| 1-Unsaturations                                                                                                | 31.2   | 35.7       |
| 2-6-Unsaturations                                                                                              | 0.7    | 3.4        |
| Total                                                                                                          | 100.0  | 100.0      |
| Total Wt % of Molecules                                                                                        | 28.3   | 26.2       |
| Having Cycloparaffinic functionality                                                                           |        |            |
| Total Wt % of Molecules Having Monocycloparaffinic functionality                                               | 27.2   | 22.8       |
| Total Wt % of Molecules Having Multicycloparaffinic functionality                                              | 0.64   | 3.4        |
| Ratio of Molecules with Monocycloparaffinic Functionality to Molecules with Multicycloparaffinic Functionality | 42.5   | 6.7        |
| SIMDIS (Wt %), ° F.                                                                                            |        |            |
| 5                                                                                                              | 847    | 804        |
| 10                                                                                                             | 856    | 887        |
| 20                                                                                                             | 869    | 973        |
| 30                                                                                                             | 881    | 991        |
| 50                                                                                                             | 905    | 1012       |
| 70                                                                                                             | 931    | 1041       |

TABLE VI-continued

| Fischer-Tropsch Derived Lubricant Base Oils |        |        |
|---------------------------------------------|--------|--------|
| Properties                                  | FT-6.4 | FT-9.7 |
| 90                                          | 962    | 1071   |
| 95                                          | 972    | 1085   |
| Boiling Range Distribution T90 – T10, ° F.  | 106    | 184    |
| Oxidator BN, hours                          | 21.3   | 12.91  |

## Example 4

The two Fischer-Tropsch derived lubricant base oils described above, and FT-4.5 described earlier, were blended with either a zinc antiwear hydraulic oil additive package designed to meet Denison HF-0 and AFNOR NFE 48-691 wet filterability standards or an ashless antiwear hydraulic oil additive package designed to meet Denison HF-0. All of these hydraulic oil blends were ISO 32 grade. The compositions and air release test results of the hydraulic oils are shown below in Table VII.

TABLE VII

| Composition of Hydraulic Oils from Co-Based Fischer-Tropsch Wax |       |       |                   |
|-----------------------------------------------------------------|-------|-------|-------------------|
| Component                                                       | Oil 5 | Oil 6 | Comparative Oil 7 |
| FT-9.7                                                          | 0     | 0     | 49.575            |
| FT-4.5                                                          | 0     | 0     | 49.575            |
| FT-6.4                                                          | 99.15 | 98.75 | 0                 |
| Zinc Antiwear HF-0 Additive Package                             | 0.85  | 0     | 0.85              |
| Ashless Antiwear HF-0 Additive Package                          | 0     | 1.25  | 0                 |
| <u>Air Release (D 3427)</u>                                     |       |       |                   |
| 50° C.                                                          | <0.1  | <0.1  | 1.13              |
| 25° C.                                                          | 0.1   | 0.1   | Not tested        |

Oils 5 and 6 both comprise: a lubricant base oil having: an average molecular weight greater than 475, a viscosity index greater than 140, less than 10 weight percent olefins; and an antiwear hydraulic oil additive.

The air release properties of Oils 5 and 6 were excellent. The excellent air release properties of these oils were related to the properties of the base oil used. In addition, the FT-6.4 base oil had a narrow boiling point distribution, a high total weight percent molecules with monocycloparaffinic functionality, a high ratio of weight percent molecules with monocycloparaffinic functionality to weight percent molecules with multicycloparaffinic functionality, and low wt % aromatics.

## Example 5

The base oils shown in Table VI are re-hydrofinished at 1000 psig to hydrogenate the olefins. As a result the wt % olefins by proton NMR in the re-hydrofinished base oils are less than 0.5 wt %. They still have average molecular weights greater than 475 and viscosity indexes greater than 140. In addition they still have greater than 10 wt % molecules with cycloparaffinic functionality, and their ratios of molecules with monocycloparaffinic functionality to weight percent molecules with multicycloparaffinic functionality are greater than 6. The oxidation stabilities of the base oils increase

dramatically, from less than 25 hours to greater than 35 hours in the Oxidator BN test. When the re-hydrofinished FT-6.4 or FT-9.7 lubricant base oils are blended with the same antiwear hydraulic oil additives as before in Oil 5 or Oil 6 and tested for air release, the air release at 50° C. is 0.5 minutes or less. The foam tendency and stability of the hydraulic oils are also very good. For example, the sequence II foam tendency by ASTM D 892-03 is less than 30 ml. In addition the oxidation stabilities of these new hydraulic oils blended with re-hydrofinished lubricant base oils are significantly better than for Oils 5 or 6.

## Example 6

A hydraulic system for mobile equipment is built. The hydraulic system has a relatively small oil reservoir; it is lighter than other similar systems; and yet it produces high power. The hydraulic system has an operating pressure of about 450 bar. The oil reservoir is factory-filled with a hydraulic oil having an air release at 50° C. by ASTM D 3427-03 of less than 0.1. The hydraulic oil also has a sequence II foam tendency by ASTM D 892-03 of less than 50 ml, and a number of minutes to 3 ml emulsion at 54° C. by ASTM D 1401-02 of less than 30.

When the hydraulic system is operated, there is no pump cavitation. The mobile equipment having the hydraulic system has an acceptably long service life.

All of the publications, patents and patent applications cited in this application are herein incorporated by reference in their entirety to the same extent as if the disclosure of each individual publication, patent application or patent was specifically and individually indicated to be incorporated by reference in its entirety.

Many modifications of the exemplary embodiments of the invention disclosed above will readily occur to those skilled in the art. Accordingly, the invention is to be construed as including all structure and methods that fall within the scope of the appended claims.

## We claim:

1. A method of operating a hydraulic pump, comprising:
  - a. filling a hydraulic system oil reservoir with a hydraulic oil comprising:
    - i. a lubricant base oil having:
      - 1) an average molecular weight greater than 475;
      - 2) a viscosity index greater than 140;
      - 3) a weight percent olefins less than 10; and
    - ii. an antiwear hydraulic oil additive package that is blended with the lubricant base oil; wherein the hydraulic oil has an air release at 50° C. by ASTM D 3427-03 of less than 0.8 minutes; and
  - b. operating the hydraulic pump supplied with the hydraulic oil from the filled oil reservoir; wherein the hydraulic pump operates without pump cavitation.
2. The method of claim 1, wherein the hydraulic pump is located in a hydraulic system of an elevator.
3. The method of claim 1, wherein the hydraulic pump is located in a hydraulic system on a mobile equipment.
4. The method of claim 3, wherein the mobile equipment is an aircraft.
5. The method of claim 3, wherein the mobile equipment is selected from the group consisting of marine equipment, forest machinery, mining machinery, agricultural machinery, construction machinery, earth moving machinery, fitness equipment, lawn and garden equipment, loading machinery, custom cars, and demolition machinery.

**21**

6. A hydraulic system, comprising a hydraulic system oil reservoir holding a hydraulic oil comprising:
- a lubricant base oil having:
    - an average molecular weight greater than 475;
    - a viscosity index greater than 140;
    - a weight percent olefins less than 10; and
  - an antiwear hydraulic oil additive package that is blended with the lubricant base oil; wherein the hydraulic oil has an air release at 50° C. by ASTM D 3427-03 of less than 0.8 minutes.
7. The hydraulic system of claim 6, wherein the air release at 50° C. is less than 0.5 minutes.
8. The hydraulic system of claim 6, wherein the hydraulic oil additionally comprises an air release at 25° C. less than 10 minutes.
9. The hydraulic system of claim 6, wherein the hydraulic oil additionally has a sequence I foam tendency by ASTM D 892-03 of less than 50 ml.
10. The hydraulic system of claim 6, wherein the hydraulic oil additionally has a sequence II foam tendency by ASTM D 892-03 of less than 30 ml.
11. The hydraulic system of claim 6, wherein the hydraulic oil meets the Denison HF-0 hydraulic oil standard.
12. The hydraulic system of claim 6, wherein the hydraulic oil is factory-filled.
13. The hydraulic system of claim 6, wherein the hydraulic system is an elevator.
14. The hydraulic system of claim 6, wherein the hydraulic system is on a mobile equipment.

**22**

15. The hydraulic system of claim 14, wherein the mobile equipment is an aircraft.
16. The hydraulic system of claim 14, wherein the mobile equipment is selected from the group consisting of marine equipment, forest machinery, mining machinery, agricultural machinery, construction machinery, earth moving machinery, fitness equipment, lawn and garden equipment, loading machinery, custom cars, and demolition machinery.
17. The hydraulic system of claim 7, additionally comprising a hydraulic pump that is supplied with the hydraulic oil from the hydraulic system oil reservoir.
18. The hydraulic system of claim 17, wherein the hydraulic system has an average operating pressure of about 300 bar to about 500 bar.
19. The hydraulic system of claim 18, wherein the hydraulic system has an average operating pressure of about 400 bar to about 475 bar.
20. A hydraulic system, comprising a hydraulic system oil reservoir holding a hydraulic oil comprising:
- a lubricant base oil, and
  - an antiwear hydraulic oil additive package that is blended with the lubricant base oil; wherein the hydraulic oil has:
    - an air release at 50° C. by ASTM D 3427-03 of less than 0.8 minutes;
    - a sequence II foam tendency by ASTM D 892-03 of less than 50 ml; and
    - a number of minutes to 3 ml emulsion at 54° C. by ASTM D 1401-02 of less than 30.

\* \* \* \* \*